

N. V. PARK.

ELECTROPLATING PROCESS.

APPLICATION FILED JULY 6, 1921.

1,423,815.

Patented July 25, 1922.



FIG. 1.



FIG. 2.

Nelson V. Park

Inventor

By William C. Linton

Attorney

# UNITED STATES PATENT OFFICE.

NELSON V. PARK, OF NILES, MICHIGAN.

## ELECTROPLATING PROCESS.

1,423,815.

Specification of Letters Patent. Patented July 25, 1922.

Application filed July 6, 1921. Serial No. 482,769.

To all whom it may concern:

Be it known that I, NELSON V. PARK, a citizen of the United States of America, residing at Niles, in the county of Berrien 5 and State of Michigan, have invented certain new and useful Improvements in Electroplating Processes; and I do hereby declare that the following is a full, clear, and exact description of the invention, such as 10 will enable others skilled in the art to which it appertains to make and use the same.

This invention has reference to improvements in electro-plating by aqueous bath having for an object, the provision of a 15 novel process for effecting the rapid decomposition of the plating metal and its transfer to the receiving body without losses of the same and without the addition of metals in chemical form with the 20 electrolyte.

It is also an object of the invention to provide a process which may be practiced at a cost materially less than that required by such methods or processes of electro-plating heretofore known in the art, and also, to permit of electro-plating in an efficient manner in materially less time than that heretofore required.

Other objects will be in part obvious and 30 in part pointed out hereinafter.

In order that the invention and its mode of application may be readily understood by persons skilled in the art, I have in the accompanying illustrative drawings and in 35 the detailed following description based thereon, set forth one embodiment of the same.

In these drawings:

Figure 1 is a sectional view, partly dia- 40 grammatic, showing the manner in which my improved electro-plating process is practiced; and,

Figure 2 is an enlarged detail in cross section through the air injecting pipe.

Having more particular reference to the drawings, in connection with which like characters of reference will designate corresponding parts, in practicing my improved process, I employ the usual electro-plating cell 1, placing therein an electrolyte or plating bath 2 and leading into 45 said cell electrical conductors 3 and 4, the conductor 3 constituting the positive side of the source of energy to which said conduc-

tors are connected (not shown) while the 55 conductor 4 constitutes the negative side thereof.

An anode 5 composed of the metal to be transferred in the plating process is supported by means of a suitable hook 6 upon 60 the positive wire 3 while a cathode 7 or the article or body which is to receive the plating metal from the anode is likewise supported as at 8 upon the negative wire 4; said anode and cathode, of course, being 65 immersed in the electrolyte 2.

A blower 9 or other suitable source of air is arranged at one side of the electro-plating cell 1 and has connection with the adjacent end of a tubular elongated nozzle 10, which, as will be noted, is formed on its lower side with a plurality of orifices 11 varying in diameter, as clearly shown in the Figure 2. It is desirable that the nozzle 10 occupy as much space as it is possible 75 in the bottom of the electro-plating cell 1 and in this connection, it may be herein noted, that if desirable, said nozzle may be provided with lateral branches or other forms of extensions, such as conditions or 80 preference may dictate, but not herein shown. It is also of importance to note that the arrangement of the orifices 11 with respect to the elongated nozzle 10 is such as to cause the directing of currents of air 85 varying in pressure downwardly towards the bottom of said electro-plating cell 1 whereby this air introduced into the electrolyte 2 will be diffused and caused to thoroughly agitate the electrolyte as a body 90 in order that the same will constantly circulate by the anode 5 and the cathode 7.

In practicing the process, current is set up in the positive and negative wires 4, 95 from a suitable source, not shown, causing electro-chemical action as between the anode and the cathode 5 and 7, respectively. This electro-chemical action results in the decomposition of metal on the anode 5 and by reason of the constantly circulating electrolyte 2, such decomposed metal will be immediately washed from the anode and transferred through the medium of the electrolyte 100 to the cathode or receiving body 7.

By injecting air into the electrolyte 2 105 through the medium of the nozzle 10 with its orifices 11 of varying diameters or sizes, it will be understood that the plating bath

will be agitated within the cell 1 and during decomposition of metal upon the anode 5, will immediately wash the same therefrom for subsequent deposit on the cathode. Thus, 5 the electrolyte is supplied with metal to its maximum carrying capacity and by consequence, because of the rapid decomposition of metal upon the anode 5 with its immediate removal therefrom to the cathode 7, the time 10 required for fully coating the cathode will be materially less than that required in heretofore practiced processes. Furthermore, the addition of metal in chemical form to maintain the strength of the plating bath is 15 entirely unnecessary, since the bath receives its supply of metal directly from the anode, which amount is ample for the cathode. Also, due to the constant washing of the anode by the electrolyte, I am enabled to 20 practically eliminate the forming of non-solvent substances, hence, requiring the use of but a small portion of chemical agents, in comparison to the amount now used in prevalent methods or processes. Furthermore, 25 by constantly washing the anode 5, the same will be practically free from any insulating substances and because of this, it will be understood that the current set up in the wires 3 and 4 may be materially reduced and yet obtain practical results.

The amount of pressure of air injected into the electrolyte 2, of course, is to be commensurate with the requirements of the work or matter to be plated, and as heretofore 35 stated, by being directed downwardly from the nozzle will serve to maintain the electrolyte in a state of constant agitation with-

out violently disturbing the same in such a manner as to cause its displacement.

To prevent the overloading of the electrolyte with the plating metal which would result in its precipitation to the bottom of the cell, the metal anode 5 is removed from the electrolyte at intervals and replaced by an anode of carbon, thus allowing the 45 amount of plating metal in the bath to be regulated to prevent waste of the same.

I claim:

1. The herein described process of electroplating which consists in introducing downwardly directed currents of air differing in pressure by means of a nozzle having openings of various diameters therein into an electrolyte containing cell having an anode and a cathode element immersed therein 55 whereby the currents of air will agitate the electrolyte and effect the continuous washing of metal from the anode for transfer to the cathode.

2. The herein described process of electroplating which consists in introducing downwardly directed currents of air differing in pressure into an electrolyte containing cell having an anode formed of the plating metal and a cathode element immersed therein 65 whereby the currents of air will agitate the electrolyte and effect the continuous washing of metal from the anode for transfer to the cathode, and replacing said metal anode, at intervals, with an anode of carbon.

In witness whereof I have hereunto set my hand.

NELSON V. PARK.